

## UNITED STATES PATENT OFFICE

2,005,747

## REMOVAL OF WOOL FROM ANIMAL SKINS

Wolf Kritchevsky, Chicago, Ill.

No Drawing. Application December 3, 1934,  
Serial No. 755,773

12 Claims. (Cl. 92—10)

My invention relates to the recovery of fur and hair from skins of animals, particularly the recovery of wool from scraps of sheepskin.

In the fur trades, scraps of sheepskin are obtained in different manufacturing and tailoring processes and this wool, if not recovered, represents a considerable economical loss. It is known that wool can be removed from sheepskin by digesting the skin with a dilute solution of sulphuric acid, thereby liberating the wool which can thereafter be treated in various ways. This process, however, is applicable to only a relatively small proportion of cases. When the skin has not been tanned at all, or when it has been aluminum tanned, the simple dilute sulphuric acid process is fairly satisfactory. On all other tanned skins, such as chrome and bark tanned skins, the simple sulphuric acid treatment heretofore known in the art will produce a wool having a dark reddish brown shade. Such a wool is almost valueless except for inferior grades of fabrics, for example, which may be left undyed or dyed very dark colors.

By my process, I treat chrome and bark tanned sheepskin and sheepskin scraps to recover a wool that is practically white and can be used in the same way that ordinary grades of wool are used in spinning, weaving and the like, and can be dyed any desirable shade without difficulty.

In my prior co-pending application, Serial No. 724,392, filed May 7, 1934, I describe a process for treating chrome and bark tanned sheepskin scraps and the like by the use of a mineral acid, employing certain features of a novel nature. While the process of my prior application involved the use of any mineral acid, it was described and had its principal advantage in connection with the use of sulphuric acid. I have now found that if I employ phosphoric acid instead of sulphuric acid, or other mineral acids, very remarkable and unexpected results are obtained, and some of the features required in the practice of the invention described in my prior application are not so essential. The manner in which the use of phosphoric acid improves the process and the respects in which features of my prior invention are either modified or deleted entirely will be apparent from a consideration of the following description.

I first prepare a solution of phosphoric acid by adding to one hundred gallons of water, one-half to two gallons of phosphoric acid of 50% strength, it being understood that more or less acid will be added depending upon its strength.

To this acid solution is added one hundred pounds

of scrap skins, the skins being boiled in the solution for a short time, or between one-half and one hour or thereabouts, until the wool or hair portion separates from the skin and the skin is substantially entirely dissolved. At this time the acid liquor is run off and the resulting wool, after washing, is found to be of a very light color, differing markedly from the wool recovered when sulphuric acid is used, principally in being of a lighter color.

While in the preferred practice of the invention using ordinary mineral acids, non-ferrous white metal scraps are added to the acid bath, this step or feature is not essential when phosphoric acid is used. I have found that in some cases the use of scrap metal in the acid bath is of some value as it has a reducing action, and the wool recovered is sometimes of a somewhat lighter color.

The wool now recovered may be further treated with a solution of a very mild alkali or alkaline product to which a reducing agent is added. While I can use an alkali wash followed by a reducing treatment as described in my prior application, very good results attend the use of a single treatment. As an example, the wool is steeped for about four or five hours in a solution of  $\frac{1}{4}\%$  of borax,  $\frac{1}{8}\%$  of soap and  $\frac{1}{4}\%$  of sodium hydro-sulphite until the wool has turned to a tan or ivory color. At this time, it is removed, washed and dried. The yield by this process is about forty pounds of wool from one hundred pounds of wool scrap.

Instead of treating the wool with the alkaline and reducing bath, it may be treated directly with a reducing agent, and a greatly improved and commercial product produced. For example, the raw wool taken from the carbonizing bath is placed in a  $\frac{1}{4}\%$  to 1% solution of hydrosulphite, or a similar reducing bath, and stirred for a short time up to several hours at luke warm or hot temperatures. The product produced by this treatment is practically colorless. The same or similar results cannot be obtained when employing sulphuric acid.

Instead of using a separate reducing bath, I may add the reducing agent directly to the carbonizing bath. This modification is not preferred, however, because too much reducing agent as a rule is required.

Still another possibility is to wash the carbonized product in an alkaline bath, as in many cases the scraps carbonized with phosphoric acid are sufficiently light in color so that a reducing bath is not necessary. In this case, a very dilute

alkaline solution is required, such as a solution with or without a buffer, such as soap. The wool may be merely rinsed in the alkaline bath, or it may be heated for some little time. In many cases, commercially satisfactory products are produced by such simple means. In general, I prefer to use an alkaline reducing bath after carbonizing, as uniform and perfect results are then assured.

10 The advantages to be secured by the use of phosphoric acid in my present process are believed fairly obvious to those skilled in the art. By using phosphoric acid as a carbonizing agent, very little color is transferred to the hair and wool, and so the hair and wool instead of coming out a dark red color after carbonizing is a very light, slightly orange brown or pinkish color, which in itself is a commercial product. In other words, this product may be washed and sold as a commercial product without further treatment. The wool obtained by the carbonizing step of my present process may be subsequently treated by an alkaline and reducing wash, and the washing can be done at a lower temperature than when sulphuric acid carbonization is used, and much more pleasing results will be obtained. Then again, a reducing step may be used after carbonization, without the use of an alkaline wash. Another advantage of the present process is that a greater 30 yield of wool is obtained with a given amount of scrap. Furthermore, since a lower temperature can be used in the alkaline wash, there is much less danger of gelatinizing the wool and in general the use of a buffer is not necessary.

35 My invention is described as taking place in a number of steps, but those skilled in the art understand that in the practical carrying on of the process, continuous operations may be used. In other words, the process lends itself to either batch 40 or continuous treatment, depending upon the type of equipment used and the convenience of either the batch or continuous treatment in a given case.

45 The invention has been described as applicable to the treatment of wool, but obviously it may be used to recover any type of animal hair or fur from scraps of skin. Indeed, it is not limited to use on scraps, but it may be used on larger pieces of wool or hair even though for commercial 50 reasons it would very seldom be used except on scraps. Although the invention is of principal value in the treatment of scraps of sheepskin, it is not limited to this specific use. The term "wool" is used in the claims, therefore, to include 55 any hair, fur, or woollike substance growing out of animal skin.

60 Although the specification sets out exact percentages and amounts of specific materials employed in the process, particularly in the examples, it is to be understood that modifications may be made and a process employed coming within the scope of the appended claims. For example, the amount of phosphoric acid used may be modified to take care of changed conditions. Where 65 sodium salts are called for, other alkali salts of the same and similar substances may be substituted. Accordingly, the details given are not by

way of limitation, but are given for the purpose of illustration and example.

What I claim as new and desire to protect by Letters Patent of the United States is:

1. The method of recovering wool from dyed animal skin, which includes the step of boiling the skin in a dilute solution of phosphoric acid. 5
2. The method of recovering wool from dyed animal skin, which includes the step of boiling the skin in a dilute solution of phosphoric acid 10 to which a non-ferrous metal in relatively finely divided form has been added.
3. The method of recovering wool from animal skin which includes the step of treating the skin with a phosphoric acid solution to free the wool 15 from the skin, and thereafter treating the wool with a dilute solution of an alkaline substance.
4. The method of recovering wool from animal skin, including the step of treating the skin with a solution of phosphoric acid to free the wool 20 from the skin, and thereafter treating the wool with a dilute solution of an alkaline substance and reducing agent.
5. The method of recovering wool from dyed animal skin, which includes the step of treating 25 the skin with a dilute solution of phosphoric acid.
6. The method of recovering wool from dyed animal skin, which includes the step of treating the skin with a dilute solution of phosphoric acid 30 to which a non-ferrous metal in relatively finely divided form has been added.
7. The method of recovering wool from animal skin which includes the step of boiling the skin in a phosphoric acid solution to free the wool 35 from the skin, and thereafter treating the wool with a dilute solution of an alkaline substance.
8. The method of recovering wool from animal skin, including the step of boiling the skin in a solution of phosphoric acid to free the wool from the skin, and thereafter treating the wool with a dilute solution of an alkaline substance and reducing agent. 40
9. The method of recovering wool from dyed animal skin which includes the step of treating the skin with a dilute solution of phosphoric acid 45 to free the wool from the skin, and thereafter treating the wool with a solution of an alkaline reacting substance.
10. The method of recovering wool from dyed animal skin which includes the step of treating the skin with a dilute solution of phosphoric acid 50 to free the wool from the skin, and thereafter treating the wool with a solution of an alkaline reacting substance and a reducing agent.
11. The method of recovering wool from animal skin which includes the step of treating the skin with a solution of phosphoric acid to free the wool from the skin, and thereafter treating the wool with a dilute solution of approximately 1/4% borax, 1/8% soap and 1/4% sodium hydro-sulphite. 55
12. The method of recovering wool from animal skin, which includes treating the skin with a solution of phosphoric acid to free the wool from the skin, and thereafter treating the wool with a reducing agent. 60

WOLF KRITCHEVSKY.